# EUROPEAN PATENT SPECIFICATION

(11) **EP 0 493 326 B1**
(45) Date of publication and mention of the grant of the patent: **25.06.1997**
(21) Application number: 91810992.7
(22) Date of filing: 20.12.1991
(51) Int. Cl.: C25B 11/00, C25C 7/02, C23C 4/02, C25D 17/10, C23C 28/00

(54) **Substrate of improved melt sprayed surface morphology**
Substrat mit verbesserter Oberflächemorphologie mittels schmelzflüssigen Spritzens
Substrat présentant une morphologie de surface améliorée par projection à l'état fondu

(30) Priority: 26.12.1990 US 633914
(43) Date of publication of application: 01.07.1992
(73) Proprietor: ELTECH SYSTEMS CORPORATION, Boca Raton Florida 33434 (US)
(72) Inventor: Ernes, Lynne M., Willoughby, Ohio 44094 (US); Carlson, Richard C., Euclid, Ohio 44123 (US); Hardee, Kenneth L., Middlefield, Ohio 44062 (US)
(74) Representative: Cronin, Brian Harold John

(56) References cited:
- EP-A- 0 275 083
- EP-A- 0 287 023
- EP-A- 0 407 349
- US-A- 2 320 329
- CHEMICAL ABSTRACTS, vol. 1111, no. 24, 11 December 1989, Columbus, Ohio, US; abstract no. 221016x, KATSURADA 'nonconsumable anode for electroplating' page 447 ;column 111 ; & JP-A-01150000

## Description

This application is a continuation-in-part of U.S. Patent Application Serial No. 374,429 filed June 30, 1989.

### Background of the Invention

The adhesion of coatings applied directly to the surface of a substrate metal is of special concern when the coated metal will be utilized in a rigorous industrial environment. Careful attention is usually paid to surface treatment and pre-treatment operation prior to coating. Achievement particularly of a clean surface is a priority sought in such treatment or pre-treatment operation.

Representative of a coating applied directly to a base metal is an electrocatalytic coating, often containing a precious metal from the platinum metal group, and applied directly onto a metal such as a valve metal. Within this technical area of electrocatalytic coatings applied to a base metal, the metal may be simply cleaned to give a very smooth surface. U.S. Patent No, 4,797,182. Treatment with fluorine compounds may produce a smooth surfacc. U.S. Patent No. 3,864,163. Cleaning might include chemical degreasing, electrolytic degreasing or treatment with an oxidizing acid. U.S. Patent 3,864,163.

Cleaning can be followed by mechanical roughening to prepare a surface for coating. U.S. Patent No, 3,778,307. If the mechanical treatment is sandblasting, such may be followed by etching. U.S. Patent No. 3,878,083. Or such may be followed by flame spray application of a fine-particled mixture of metal powders. U.S. Patent No. 4,849,085.

Another procedure for anchoring the fresh coating to the substrate, that has found utility in the application of an electrocatalytic coating to a valve metal, is to provide a porous oxide layer which can be formed on the base metal. For example, titanium oxide can be flame or plasma sprayed onto substrate metal before application of electrochemically active substance, as disclosed in U.S. Patent No. 4,140,813. Or the thermally sprayed material may consist of a metal oxide or nitride or so forth, to which electrocatalytically active particles have been pre-applied, as taught in U.S. Patent No. 4,392,927.

It has however been found difficult to provide long-lived coated metal articles for serving in the most rugged commercial environments, e.g., oxygen evolving anodes for use in the present-day commercial applications utilized in electrogalvanizing, electrotinning, electroforming or electrowinning. Such may be continuous operation. They can involve severe conditions including potential surface damage. It would be most desirable to provide coated metal substrates to serve as electrodes in such operations, exhibiting extended stable operation while preserving excellent coating adhesion. It would also be highly desirable to provide such an electrode not only from fresh metal but also from recoated metal.

### Summary of the Invention

There has now been found a metal surface which provides a locked on coating of excellent coating adhesion. The coated metal substrate can have highly desirable extended lifetime even in most rigorous industrial environments. For the electrocatalytic coatings, the invention can provide for well anchored coatings of uniform planarity, even when utilizing gouged and similarly disfigured substrate metal.

In one aspect, the invention is directed to a method of producing a metallic article comprising a substrate having a metal-containing surface adapted for enhanced coating adhesion by melt spraying valve metal particles having a size within the range from 20 to 100 micrometers to produce a surface having a profilometer-measured average surface roughness of about 6.35 micrometers (about 250 microinches), or more, and an average surface peaks per cm of about 15.7 (about 40 peaks per inch), or more, basis a profilometer upper threshold limit of 10.16 micrometers (400 microinches) and a profilometer lower threshold limit of 7.62 micrometers (300 microinches).

In another aspect, the invention is directed to the method of preparing a metal surface for enhanced coating adhesion which surface has been gouged and thereby exhibits loss of planarity, which method comprises: plasma spraying the gouges of such surface with a valve metal to establish metal surface planarity, and then plasma spraying the surface to be coated, including the plasma sprayed gouges to provide a surface roughness of enhanced coating adhesion, as defined above.

In a still further aspect, the invention is directed to a metallic article coated with an intermediate layer and an electrochemically active surface coating, particularly for use as an electrode in electrochemical processes. When the metal articles are electrocatalytically coated and used as oxygen evolving electrodes, even under the rigorous commercial operations including continuous electrogalvanizing, electrotinning, copper foil plating, electroforming or electrowinning, and including sodium sulfate electrolysis such electrodes can have highly desirable service life. Thus the invention is also directed to such metal articles as are utilized as electrodes.

### Description of the Preferred Embodiments

The metals of the substrate are broadly contemplated to be any coatable metal. For the particular application of an electrocatalytic coating, the substrate metals might be such as nickel or manganese, but will most always be valve metals, including titanium, tantalum, aluminum, zirconium and niobium. Of particular interest for its ruggedness, corrosion resistance and availability is titanium. As well as the normally available elemental metals themselves, the suitable metals of the substrate can include metal alloys and intermetallic mixtures, as well as ceramics and cermets such as contain one or more valve metals. For example, titanium may be alloyed with nickel, cobalt, iron, manganese or copper. More specifically, Grade 5 titanium may include up to 6.75 weight% aluminum and 4.5 weight% vanadium, grade 6 up to 6% aluminum and 3% tin, grade 7 up to 0.25 weight% palladium, grade 10, from 10 to 13 weight% molybdenum plus 4.5 to 7.5 weight% zirconium and so on.

By use of elemental metals, alloys and intermetallic mixtures, it is most particularly meant the metals in their normally available condition, i.e., having minor amounts of impurities. Thus for the metal of particular interest, i.e., titanium, various grades of the metal are available including those in which other constituents may be alloys or alloys plus impurities. Grades of titanium have been more specifically set forth in the standard specifications for titanium detailed in ASTM B 265-79.

Regardless of the metal selected and how the metal surface is subsequently processed, the substrate metal advantageously is a cleaned surface. This may be obtained by any of the treatments used to achieve a clean metal surface, but with the provision that unless called for to remove an old coating, and if etching might be employed, as more specifically detailed hereinbelow, mechanical cleaning is typically minimized. Thus the usual cleaning procedures of degreasing, either chemical or electrolytic, or other chemical cleaning operation may be used to advantage.

Where an old coating is present on the metal surface, such needs to be addressed before recoating. It is preferred for best extended performance when the finished article will be used with an electrocatalytic coating, such as use as an oxygen evolving electrode, to remove the old coating. In the technical area of the invention which pertains to electrochemically active coatings on a valve metal, chemical means for coating removal are well known. Thus a melt of essentially basic material, followed by an initial pickling will suitably reconstitute the metal surface, as taught in U.S. Patent No. 3,573,100. Or a melt of alkali metal hydroxide containing alkali metal hydride, which may be followed by a mineral acid treatment, is useful, as described in U.S. Patent No. 3,706,600. Usual rinsing and drying steps can also form a portion of these operations.

When a cleaned surface, or prepared and cleaned surface has been obtained, and particularly for later applying an electrocatalytic coating to a valve metal in the practice of the present invention, surface roughness is then obtained. This will be achieved by means which include plasma spray application, usually of particulate valve metal, most especially titanium powder. However, as described hereinbelow, although the metal will be applied in particulate form, the feed metal, i.e., the metal to be applied, may be in different form such as wire form. This should be understood even though for convenience, application will typically be discussed as metal applied in particulate form. In this plasma spraying, the metal is melted and sprayed in a plasma stream generated by heating with an electric arc to high temperatures an inert gas, such as argon or nitrogen, optionally containing a minor amount of hydrogen. It is to be understood by the use herein of the term "plasma spraying" that although plasma spraying is preferred the term is meant to include generally thermal spraying such as magnetohydrodynamic spraying, flame spraying and arc spraying, generally referred to as melt spraying.

The spraying parameters, such as the volume and temperature of the flame or plasma spraying stream, the spraying distance, the feed rate of particulate metal constituents and the like, are chosen so that the particulate metal components are melted by and in the spray stream and deposited on the metal substrate while still substantially in melted form so as to provide an essentially continuous coating (i.e. one in which the sprayed particles are not discernible) having a foraminous structure. Typically, spray parameters like those used in the examples give satisfactory coatings. Usually, the metal substrate during melt spraying is maintained near ambient temperature. This may be achieved by means such as streams of air impinging on the substrate during spraying or allowing the substrate to air cool between spray passes.

The particulate metal employed, e.g., titanium powder, has a typical particle size range of 20 - 100 micrometers, and preferably has all particles within the range of 40 - 80 micrometers for efficient preparation of surface roughness. The metallic constituency of the particulates may be as above-described for the metals of the substrate, e.g., the titanium might be one of several grades most usually grade 1 titanium. It is also contemplated that mixtures may be applied, e.g., mixtures of metals or of metals with other subsituents, which can include metal oxides, for example a predominant amount of metal with a minor amount of other substituents.

It is also contemplated that such plasma spray applications may be used in combination with etching of the substrate metal surface, with each treatment most always being applied to different portions of a surface. If etching is used, it is important to aggressively etch the metal surface to provide deep grain boundaries and well exposed, three-dimensional grains. It is preferred that such operation will etch impurities located at such grain boundaries.

Particularly where an old coating has been present and the coated substrate has been in use, e.g., as an anode in electrogalvanizing, the metal article can be disfigured and can have lost surface planarity. Typically, such disfiguring will be in nicks and gouges of the surface. For convenience, all such surface disfigurement, including nicks, scrapes, and gouges, and burns where metal may actually be melted and resolidify, will generally be referred to herein simply as "gouges." These may or may not be filled with a metal filling. If the overall surface were to be subsequently etched before recoating, the filled zones can be expected to yield poor etch results. Also, gouging of the substrate may be extensive, or the substrate from its heat history and/or chemistry may not achieve desirable results in etching. It may, therefore, be especially desirable to simply plasma spray the entire surface which can overcome these substrate deficiencies. It is also contemplated that it may be useful to combine plasma spray application with etching in some situations. Thus, gouges and the like may be filled by plasma spray technique. Usually, the areas of the surface which are not disfigured will first be etched, then the planar, etched areas can be masked, and the gouges remaining will be filled and/or surface treated by plasma spray application. That is, plasma spray can be used to fill and reactivate a gouge, or it simply can be used to just reactivate gouges without necessarily restoring surface planarity. By reactivation is meant the plasma spray application to prepare the gouge for subsequent treatment. Hence, the entire surface will have the needed roughness for coating, and if desired it may in the same processing be refurbished to desirable planarity.

When etching is utilized the heat treatment history of the metal can be important. For example, to prepare a metal such as titanium for etching, it can be most useful to condition the metal, as by annealing, to diffuse impurities to the grain boundaries. Thus, by way of example, proper annealing of grade 1 titanium will enhance the concentration of the iron impurity at grain boundaries. Where the suitable preparation includes annealing, and the metal is grade 1 titanium, the titanium can be annealed at a temperature of at least about 500°C. for a time of at least about 15 minutes. For efficiency of operation, a more elevated annealing temperature, e.g., 600°-800°C. is advantageous.

Where etching is employed, it will be with a sufficiently active etch solution to develop aggressive grain boundary attack. Typical etch solutions are acidic solutions. These can be provided by hydrochloric, sulfuric, perchloric, nitric, oxalic, tartaric, and phosphoric acids as well as mixtures thereof, e.g., aqua regia. Other etchants that may be utilized include caustic etchants such as a solution of potassium hydroxide/hydrogen peroxide in combination, or a melt of potassium hydroxide with potassium nitrate. For efficiency of operation, the etch solution is advantageously a strong, or concentrated solution such as an 18-22 weight% solution of hydrochloric acid. Moreover, the solution is advantageously maintained during etching at elevated temperature such as at 80°C. or more for aqueous solutions, and often at or near boiling condition or greater, e.g., under refluxing condition. Following etching, the etched metal surface can then be subjected to rinsing and drying steps to prepare the surface for coating. A more detailed discussion of the etching and annealing can be found in EP-A-0 407 349.

For the plasma spray applied surface roughness, it is necessary that the metal surface have an average roughness (Ra) about 6.35 micrometers (about 250 microinches), or more, and an average number of surface peaks per cm (Nr) of at least about 15.7 (about 40 peaks per inch). The surface peaks per cm can be typically measured at a lower threshold limit of 7.62 micrometers (300 microinches) and an upper threshold limit of 10.16 micrometers (400 microinches). A surface having an average roughness of below about 6.35 micrometers (about 250 microinches) will be undesirably smooth, as will a surface having an average number of surface peaks per cm of below about 15.7 (about 40 peaks per inch) for providing the needed, substantially enhanced, coating adhesion. Advantageously, the surface will have an average roughness of on the order of about 10.16 micrometers (about 400 microinches) or more, e.g., ranging up to about 19-38.1 micrometers (about 750-1500 microinches), with no low spots of less than about 5.08 micrometers (about 200 microinches). Advantageously, for best avoidance of surface smoothness, the surface will be free from low spots that are less than about 5.33 to 5.59 micrometers (about 210 to 220 microinches). It is preferable that the surface have an average roughness of from about 7.62 to 12.7 micrometers (about 300 to about 500 microinches). Advantageously, the surface has an average number of peaks per cm of at least about 23.25 (about 60 peaks per inch), but which might be on the order of as great as about 130 or more, with an average from about 80 to about 120 being preferred. It is further advantageous for the surface to have an average distance between the maximum peak and the maximum valley (Rm) of at least about 25.37 µm (1,000 microinches) and to have an average peak height (Rz) of at least about 25.37 µm (1,000 microinches). All of such foregoing surface characteristics are as measured by a profilometer. More desirably, the surface for coating will have an Rm value of at least about 38.1 µm (1,500 microinches) to about 53.34 µm (3500 microinches) and have a maximum valley characteristic of at least about 38.1 µm (1,500 microinches) up to about 53.34 µm (3500 microinches).

After the substrate has attained the necessary surface roughness, it will be understood that the surface may then proceed through various operations, including pretreatment before coating. For example, the surface may be subjected to a cleaning operation, e.g., a solvent wash. Or it may be subjected to a subsequent etching or hydriding or nitriding treatment. Prior to coating with an electrochemically active material, it has been proposed to provide an oxide layer by heating the substrate in air or by anodic oxidation of the substrate as described in U.S. Patent No. 3,234,110. European patent application No. 0,090,425 proposes to platinum electroplate the substrate to which then an oxide of ruthenium, palladium or iridium is chemideposited. Various proposals have also been made in which an outer layer of electrochemically active material is deposited on a sub-layer which primarily serves as a protective and conductive intermediate. U.K. Patent No. 1,344,540 discloses utilizing an electrodeposited layer of cobalt or lead oxide under a ruthenium-titanium oxide or similar active outer layer. Various tin oxide based underlayers are disclosed in U.S. Patents No, 4,272,354, 3,882,002 and 3,950,240. After providing the necessary surface roughness followed by any pretreatment operation, the coating most contemplated in the present invention is the application of electrochemically active coating.

As representative of the electrochemically active coatings that may then be applied to the etched surface of the metal, are those provided from platinum or other platinum group metals or they can be represented by active oxide coatings such as platinum group metal oxides, magnetite , ferrite, cobalt spinel or mixed metal oxide coatings. Such coatings have typically been developed for use as anode coatings in the industrial electrochemical industry. They may be water based or solvent based, e.g., using alcohol solvent. Suitable coatings of this type have been generally described in one or more of the U.S. Patent Nos. 3,265,526, 3,632,498, 3,711,385 and 4,528,084. The mixed metal oxide coatings can often include at least one oxide of a valve metal with an oxide of a platinum group metal including platinum, palladium, rhodium, iridium and ruthenium or mixtures of themselves and with other metals. Further coatings in addition to those enumerated above include manganese dioxide, lead dioxide, platinate coatings such as MₓPt₃O₄ where M is an alkali metal and X is typically targeted at approximately 0.5, nickel-nickel oxide and nickel plus lanthanide oxides.

It is contemplated that coatings will be applied to the metal by any of those means which are useful for applying a liquid coating composition to a metal substrate. Such methods include dip spin and dip drain techniques, brush application, roller coating and spray application such as electrostatic spray. Moreover spray application and combination techniques, e.g., dip drain with spray application can be utilized. With the above-mentioned coating compositions for providing an electrochemically active coating, a modified dip drain operation can be most serviceable. Following any of the foregoing coating procedures, upon removal from the liquid coating composition, the coated metal surface may simply dip drain or be subjected to other post coating technique such as forced air drying.

Typical curing conditions for electrocatalytic coatings can include cure temperatures of from about 300°C. up to about 600°C. Curing times may vary from only a few minutes for each coating layer up to an hour or more, e.g., a longer cure time after several coating layers have been applied. However, cure procedures duplicating annealing conditions of elevated temperature plus prolonged exposure to such elevated temperature, are generally avoided for economy of operation. In general, the curing technique employed can be any of those that may be used for curing a coating on a metal substrate. Thus, oven curing, including conveyor ovens may be utilized. Moreover, infrared cure techniques can be useful. Preferably for most economical curing, oven curing is used and the cure temperature used for electrocatalytic coatings will be within the range of from about 450°C. to about 550°C. At such temperatures, curing times of only a few minutes, e.g., from about 3 to 10 minutes, will most always be used for each applied coating layer.

The following examples show ways in which the invention has been practiced, as well as showing comparative examples. However, the examples showing ways in which the invention has been practiced should not be construed as limiting the invention.

### EXAMPLE 1

A titanium nut is welded to the back of each sample plate having an approximate 7.5 cm² sample face and each being unalloyed grade 1 titanium. The sample plates were then mounted to a large back plate to provide a mosaic of sample plates. This mounting scheme served to provide a large array of sample plates which could be handled as a unit in ensuing operations. The sample plates were grit blasted with aluminum oxide, then rinsed in acetone and dried.

A coating on the sample plates of titanium powder was produced using a powder having average particle size of 50 - 60 µm (microns). The sample plates were coated with this powder using a Metco plasma spray gun equipped with a GH spray nozzle. The spraying conditions were: a current of 500 amps; a voltage of 45 - 50 volts; a plasma gas consisting of argon and helium; a titanium feed rate of 1.36 kg (3 pounds) per hour; a spray bandwidth of 6.7 millimeters (mm); and a spraying distance of 64 mm, with the resulting titanium layer on the titanium sample plates having a thickness of about 150 micrometers.

The coated surface of the sample plates were then subjected to surface prolifilometer measurement using a Hommel model T1000 C instrument manufactured by Hommelwerk GmbH. The plate surface profilometer measurements were determined from three separate measurements conducted by running the instrument in random orientation across the coated flat face of the plate. This gave average values as measured on three sample plates for surface roughness (Ra) of 11.38, 12.45 and 13.9 micrometers (448, 490 and 548 microinches), respectively for the three plates, and peaks per cm (Nr) of 29.8, 24.7 and 29.8 (76, 63 and 76 peaks per inch), respectively for the three plates. The peaks per cm were measured within the threshold limits of 7.62 micrometers (300 microinches) (lower) and 10.16 micrometers (400 microinches) (upper).

### EXAMPLE 2

A sample of titanium which had been previously coated with an electrochemically active coating, was blasted with alumina powder to remove the previous coating. By this abrasive method, it was determined by X-ray fluorescence that the previous coating had been removed. Aster removal of any residue of the abrasive treatment, the resulting sample plate was etched. It was etched for approximately 1 hours by immersion in 20 weight percent hydrochloric acid aqueous solution heated to 95°C. After removal from the hot hydrochloric acid, the plate was again rinsed with deionized water and air dried. Under profilometer measurement conducted in the manner of Example 1, the resulting average values for a flat face surface of the sample were found to be 180 (Ra) and 31 (Nr).

The sample then received a coating of plasma spray applied titanium using the titanium powder and the application procedure as described in Example 1. Under profilometer measurement conducted in the manner of Example 1, the resulting average values for a flat surface of the sample were found to be 650 (Ra) and 69 (Nr).

## Claims

1. A method of producing a metallic article comprising a substrate having a metal-containing surface adapted for enhanced coating adhesion by melt spraying valve metal particles having a size within the range from 20 to 100 micrometers to produce a surface having a profilometer-measured average surface roughness of about 6.35 micrometers (about 250 microinches), or more, and an average surface peaks per cm of about 15.7 (about 40 peaks per inch), or more, basis a profilometer upper threshold limit of 10.16 micrometers (400 microinches) and a profilometer lower threshold limit of 7.62 micrometers (300 microinches).

2. The method of claim 1, wherein the substrate comprises a valve metal as one or more of a metal, alloy, intermetallic mixture, ceramic or cermet.

3. The method of claim 1 or 2, wherein the melt-sprayed metal of said surface is selected from the metals, alloys, and intermetallic mixtures of titanium, tantalum, niobium, aluminium, zirconium, manganese and nickel.

4. The method of claim 3, wherein said metal surface has a profilometer-measured average roughness of about 7.62 micrometers (about 300 microinches), or more, with no low spots of less than about 5.33 micrometers (about 210 microinches).

5. The method of any preceding claim, wherein said surface has a profilometer-measured average surface peaks per cm of at least about 23.6 (about 60 peaks per inch), basis an upper threshold limit of 10.16 micrometers (400 microinches) and a lower threshold limit of 7.62 micrometers (300 microinches).

6. The method of any preceding claim, wherein said surface has profilometer-measured average distance between the maximum peak and the maximum valley of at least about 25.4 micrometers (about 1000 microinches).

7. The method of claim 6, wherein said surface has profilometer-measured average distance between the maximum peak and the maximum valley of about 38.1 micrometers (about 1500 microinches) to about 88.9 micrometers (about 3500 microinches).

8. The method of any preceding claim, wherein said surface has a profilometer-measured average peaks height of about 25.4 micrometers (about 1000 microinches) or more.

9. The method of claim 8, wherein said surface has a profilometer-measured average peaks height of from about 38.1 micrometers (about 1500 microinches) to about 88.9 micrometers (about 3500 microinches).

10. The method of any preceding claim, wherein said surface is coated.

11. The method of claim 10, wherein said surface is coated with an electrochemically active surface coating containing a platinum group metal, or a metal oxide or their mixtures, in particular a mixed crystal material of at least one oxide of a valve metal and at least one oxide of a platinum group metal.

12. The method of claim 11, wherein said electrochemically active surface coating contains at least one oxide selected from the platinum group metal oxides, magnetite, ferrite, and cobalt oxide spinel, manganese dioxide, lead dioxide, tin oxide, platinate substituent, nickel-nickel oxide and nickel plus lanthanide oxides.

13. The method of claim 11 or 12, wherein prior to applying the electrochemically active surface coating, an oxide hydride or nitride layer is produced on the melt-sprayed surface.

14. The method of claim 11 or 12, wherein prior to applying the electrochemically active surface coating a protective and conductive intermediate sub-layer such as electroplated platinum, electrodeposited cobalt oxide or lead oxide, or a tin-oxide based layer is applied on the plasma-sprayed surface.

15. The method of any preceding claim, for producing an electrode for electrochemical processes, especially an oxygen-evolving anode.

16. The method of claim 15, for producing an anode in an anodizing, electroplating or electrowinning cell.

17. The method of claim 15, for producing an anode in electrogalvanizing, electrotinning, sodium sulfate electrolysis or copper foil plating.

18. The method of preparing a planar metal surface for enhanced coating adhesion, which surface has been gouged and thereby exhibits loss of planarity, which method comprises :
a) melt spraying the gouges of said surface with a valve metal, preferably by plasma spraying, to establish metal surface planarity, and then
b) melt spraying the surface to be coated, including the melt sprayed gouges, preferably with the same valve metal as before and preferably by plasma spraying, with particles having a size within the range from 20 to 100 micrometers to provide a surface roughness of enhanced coating adhesion, as defined in claim 1.

19. The method of claim 18, wherein said gouges are first partially filled with weld material and then melt sprayed with valve metal.

20. The method of claim 18 or 19, wherein said gouges are first milled to provide milled gouges for melt spray applied metal.

21. The method of preparing a surface of a coated metal in planar shape for recoating, which surface has been gouged in use and exhibits loss of planarity, which method comprises :
a) subjecting said coated metal surface to a melt containing molten material for removing said coating, preferably by dipping the coated metal surface in said melt;
b) separating said metal surface from said melt, cooling same and removing melt residue therefrom;
c) etching intergranularly the surface at an elevated temperature and with a strong acid or caustic etchant;
d) washing said etched surface exposing said gouges; and
e) melt spraying the gouges of said surface with particles of a valve metal having a size within the range from 20 to 100 micrometers, preferably by plasma spraying, to establish metal surface planarity and provide surface roughness; and
f) whereby said surface has surface planarity plus surface roughness for enhanced coating adhesion, as defined in claim 1, and said surface roughness is established by both intergranular etching and plasma spraying.

22. The method of claim 21, wherein said surface separated from said coating-removal melt is subjected to elevated temperature annealing for a time sufficient to provide an at least substantially continuous intergranular network of impurities, including impurities at the surface of said metal.

23. The method of claim 21 or 22, wherein said gouges are first partially filled with weld material and then melt sprayed with valve metal, preferably by plasma spraying.

24. The method of claim 23, wherein said gouges are first milled to provide milled gouges for melt-spray applied valve metal.

25. A coated metallic article comprising :
- a substrate having a metal-containing surface adapted for enhanced coating adhesion, said surface comprising a melt spray applied valve metal surface on the substrate, which surface is applied by melt spraying valve metal particles having a size within the range from 20 to 100 micrometers and has a profilometer-measured average surface roughness of about 6.35 micrometers (about 250 microinches), or more, and an average surface peaks per cm of about 15.7 (about 40 peaks per inch), or more, basis a profilometer upper threshold limit of 10.16 micrometers (400 microinches) and a profilometer lower threshold limit of 7.62 micrometers (300 microinches);
- a conductive intermediate layer which is an oxide layer produced by oxidizing the melt-sprayed valve metal surface by heating in air or by anodic oxidation, or a hydride or nitride layer produced by subjecting the melt-sprayed valve metal surface to a hydriding or nitriding treatment; or is a protective and conductive sub-layer applied onto the melt-sprayed valve metal surface; and
- an electrochemically active surface coating.

26. The article of claim 25, wherein the substrate comprises a valve metal as one or more of a metal, alloy, intermetallic mixture, ceramic or cermet.

27. The article of claim 25 or 26, wherein the melt-sprayed metal of said surface is selected from the metals, alloys, and intermetallic mixtures of titanium, tantalum, niobium, aluminium, zirconium, manganese and nickel.

28. The article of claim 27, wherein said metal surface has a profilometer-measured average roughness of about 7.62 micrometers (about 300 microinches), or more, with no low spots of less than about 5.33 micrometers (about 210 microinches).

29. The article of any one of claims 25 to 28, wherein said surface has a profilometer-measured average surface peaks per cm of at least about 23.6 (about 60 peaks per inch), basis an upper threshold limit of 10.16 micrometers (400 microinches) and a lower threshold limit of 7.62 micrometers (300 microinches).

30. The article of any one of claims 25 to 29, wherein said surface has profilometer-measured average distance between the maximum peak and the maximum valley of at least about 25.4 micrometers (about 1000 microinches).

31. The article of claim 30, wherein said surface has profilometer-measured average distance between the maximum peak and the maximum valley of about 38.1 micrometers (about 1500 microinches) to about 88.9 micrometers (about 3500 microinches).

32. The article of any one of claims 25 to 31, wherein said surface has a profilometer-measured average peaks height of about 25.4 micrometers (about 1000 microinches) or more.

33. The article of claim 32, wherein said surface has a profilometer-measured average peaks height of from about 38.1 micrometers (about 1500 microinches) to about 88.9 micrometers (about 3500 microinches).

34. The article of any one of claims 25 to 33, wherein the intermediate layer is an oxide layer produced in the melt-sprayed surface by heating in air or by anodic oxidation.

35. The article of any one of claims 25 to 33, wherein the intermediate layer is an applied sublayer selected from electroplated platinum, electrodeposited cobalt oxide or lead oxide, or a tin-oxide based layer.

36. The article of any one of claims 25 to 35, which is an electrode for electrochemical processes, especially an oxygen-evolving anode.

37. The article of claim 36, which is an anode in an anodizing, electroplating or electrowinning cell.

38. The article of claim 36, which is an anode in electrogalvanizing, electrotinning, sodium sulfate electrolysis or copper foil plating.

39. A cell for the electrolysis of a dissolved species contained in a bath of said cell and having immersed in said bath an anode which is a coated metallic article as claimed in any one of claims 25 to 38.

## Patentansprüche

1. Verfahren zur Herstellung eines metallischen Gegenstandes, der ein Substrat umfaßt, das eine metall-enthaltende Oberfläche aufweist, die für eine erhöhte Beschichtungshaftung ausgelegt ist, bei dem Ventilmetallteilchen mit einer Größe im Bereich von 20 bis 100 µm schmelzgesprüht werden, um eine Oberfläche mit einer mittels Profilometer gemessenen durchschnittlichen Oberflächenrauheit von etwa 6,35 µm (etwa 250 Mikroinch) oder mehr und einem Durchschnitt von Oberflächenpeaks/cm von etwa 15,7 (etwa 40 Peaks/Inch) oder mehr, auf Basis einer oberen Profilometerschwellengrenze von 10,16 µm (400 Mikroinch) und einer unteren Profilometerschwellengrenze von 7,62 µm (300 Mikroinch) herzustellen.

2. Verfahren nach Anspruch 1, bei dem das Substrat ein Ventilmetall wie eines oder mehrere von einem Metall, einer Legierung, einer intermetallischen Mischung, einer Keramik oder einem Cermet umfaßt.

3. Verfahren nach Anspruch 1 oder 2, bei dem das schmelzgesprühte Metall der Oberfläche ausgewählt ist aus den Metallen, Legierungen und intermetallischen Mischungen von Titan, Tantal, Niob, Aluminium, Zirkonium, Mangan und Nickel.

4. Verfahren nach Anspruch 3, bei dem die Metalloberfläche eine mittels Profilometer gemessene durchschnittliche Rauheit von etwa 7,62 µm (etwa 300 Mikroinch) oder mehr ohne niedrige Stellen von weniger als etwa 5,33 µm (etwa 210 Mikroinch) aufweist.

5. Verfahren nach einem der vorhergehenden Ansprüche, bei dem die Oberfläche einen mittels Profilometer gemessenen Durchschnitt von Oberflächenpeaks/cm von mindestens etwa 23,6 (etwa 60 Peaks/Inch), auf Basis einer oberen Schwellengrenze von 10,16 µm (400 Mikroinch) und einer unteren Schwellengrenze von 7,62 µm (300 Mikroinch), aufweist.

6. Verfahren nach einem der vorhergehenden Ansprüche, bei dem die Oberfläche einen mittels Profilometer gemessenen durchschnittlichen Abstand zwischen dem Maximumpeak und dem Maximumtal von mindestens etwa 25,4 µm (etwa 1000 Mikroinch) aufweist.

7. Verfahren nach Anspruch 6, bei dem die Oberfläche einen mittels Profilometer gemessenen durchschnittlichen Abstand zwischen dem Maximumpeak und dem Maximumtal von etwa 38,1 µm (etwa 1500 Mikroinch) bis etwa 88,9 µm (etwa 3500 Mikroinch) aufweist.

8. Verfahren nach einem der vorhergehenden Ansprüche, bei dem die Oberfläche eine mittels Profilometer gemessenen durchschnittliche Peakhöhe von etwa 25,4 µm (etwa 1000 Mikroinch) oder mehr aufweist.

9. Verfahren nach Anspruch 8, bei dem die Oberfläche eine mittels Profilometer gemessene durchschnittliche Peakhöhe von etwa 38,1 µm (etwa 1500 Mikroinch) bis etwa 88,9 µm (etwa 3500 Mikroinch) aufweist.

10. Verfahren nach einem der vorhergehenden Ansprüche, bei dem die Oberfläche beschichtet ist.

11. Verfahren nach Anspruch 10, bei dem die Oberfläche mit einer elektrochemisch aktiven Oberflächenbeschichtung beschichtet ist, die ein Platingruppemetall oder ein Metalloxid oder deren Mischungen enthält, insbesondere ein gemischtes Kristallmaterial aus mindestens einem Oxid eines Ventilmetalls und mindestens einem Oxid eines Platingruppemetalls.

12. Verfahren nach Anspruch 11, bei dem die elektrochemisch aktive Oberflächenbeschichtung mindestens ein Oxid ausgewählt aus den Platingruppemetalloxiden, Magnetit, Ferrit und Kobaltoxidspinell, Mangandioxid, Bleidioxid, Zinnoxid, Platinatsubstituent, Nickel-Nickeloxid und Nickel plus Lanthanoxiden enthält.

13. Verfahren nach Anspruch 11 oder 12, bei dem vor der Aufbringung der elektrochemisch aktiven Oberflächenbeschichtung eine Oxid-, Hydrid- oder Nitridschicht auf der schmelzgesprühten Oberfläche erzeugt wird.

14. Verfahren nach Anspruch 11 oder 12, bei dem vor der Aufbringung der elektrochemischen aktiven Oberflächenbeschichtung eine schützende und leitfähige Zwischenunterschicht wie beispielsweise elektroplattiertes Platin, elektroabgelagertes Kobaltoxid oder Bleioxid oder eine auf Zinnoxid basierende Schicht auf die plasma-gesprühte Oberfläche aufgebracht wird.

15. Verfahren nach einem der vorhergehenden Ansprüche zur Herstellung einer Elektrode für elektrochemische Verfahren, insbesondere eine sauerstoffentwickelnde Anode.

16. Verfahren nach Anspruch 15 zur Herstellung einer Anode in einer anodisierenden elektroplattierenden oder elektrolytischen Gewinnungszelle.

17. Verfahren nach Anspruch 15 zur Herstellung einer Anode zum Elektrogalvanisieren, Elektroverzinnen, zur Natriumsulfatelektrolyse oder Kupferfolienplattierung.

18. Verfahren zur Herstellung einer planaren Metalloberfläche für eine erhöhte Beschichtungshaftung, wobei die Oberfläche ausgehöhlt worden ist und dadurch einen Verlust an Planarität zeigt, bei dem:
a) die Höhlungen der Oberfläche mit einem Ventilmetall schmelzgesprüht werden, vorzugsweise durch Plasmasprühen, um eine Metalloberflächenplanarität zu bilden, und dann
b) die zu beschichtende Oberfläche, einschließlich der schmelzgesprühten Höhlungen vorzugsweise mit dem gleichen Ventilmetall wie zuvor vorzugsweise durch Plasmasprühen mit Teilchen mit einer Größe innerhalb des Bereichs von 20 bis 100 µm schmelzgesprüht wird, um eine Oberflächenrauheit mit erhöhter Beschichtungshaftung gemäß Anspruch 1 zu liefern.

19. Verfahren nach Anspruch 18, bei dem die Höhlungen zuerst teilweise mit Schweißmaterial gefüllt werden und dann mit Ventilmetall schmelzgesprüht werden.

20. Verfahren nach Anspruch 18 oder 19, bei dem die Höhlungen zuerst gefräst werden, um gefräste Höhlungen für mittels Schmelzsprühen aufgebrachtes Metall zu liefern.

21. Verfahren zur Herstellung einer Oberfläche aus beschichtetem Metall in planarer Gestalt zur erneuten Beschichtung, wobei die Oberfläche durch Gebrauch ausgehöhlt worden ist und einen Verlust an Planarität zeigt, bei dem
a) die beschichtete Metalloberfläche einer Schmelze, die geschmolzenes Material enthält, zur Entfernung dieser Beschichtung ausgesetzt wird, vorzugsweise durch Eintauchen der beschichteten Metalloberfläche in die Schmelze,
b) die Metalloberfläche von der Schmelze getrennt wird, sie abgekühlt wird und der Schmelzrückstand davon entfernt wird,
c) die Oberfläche bei einer erhöhten Temperatur und mit einer starken Säure oder einem kaustischen Ätzmittel intergranular geätzt wird,
d) die geätzte Oberfläche gewaschen wird, was die Aushöhlungen freilegt, und
e) die Aushöhlungen der Oberfläche mit Teilchen eines Ventilmetalls mit einer Größe im Bereich von 20 bis 100 µm, vorzugsweise durch Plasmasprühen schmelzgesprüht werden, um eine Metalloberflächenplanarität herzustellen und Oberflächenrauheit zu liefern, und
f) wobei die Oberfläche eine Oberflächenplanarität plus Oberflächenrauheit für eine erhöhte Beschichtungshaftung gemäß Anspruch 1 aufweist und die Oberflächenrauheit sowohl durch intergranulares Ätzen als auch durch Plasmasprühen erzeugt wird.

22. Verfahren nach Anspruch 21, bei dem die Oberfläche, die von der Beschichtungs-entfernenden Schmelze getrennt worden ist, einem Glühen bei erhöhter Temperatur für einen Zeitraum ausgesetzt wird, der ausreicht, um mindestens ein im wesentlichen kontinuierliches intergranulares Netzwerk von Verunreinigungen, einschließlich Verunreinigungen an der Oberfläche des Metalls zu liefern.

23. Verfahren nach Anspruch 21 oder 22, bei dem die Aushöhlungen zuerst teilweise mit Schweißmaterial gefüllt werden und dann mit Ventilmetall, vorzugsweise durch Plasmasprühen schmelzgesprüht werden.

24. Verfahren nach Anspruch 23, bei dem die Aushöhlungen zuerst gefräst werden, um gefräste Aushöhlungen für mittels Schmelzsprühen aufgebrachtes Ventilmetall zu liefern.

25. Beschichteter metallischer Gegenstand, der:
- ein Substrat mit einer Metall-enthaltenden Oberfläche, die für erhöhte Beschichtungshaftung ausgelegt ist, wobei die Oberfläche eine mittels Schmelzsprühen aufgebrachten Ventilmetalloberfläche auf dem Substrat umfaßt, die durch Schmelzsprühen von Ventilmetallteilchen mit einer Größe im Bereich von 20 bis 100 µm aufgebracht worden ist und eine mittels Profilometer gemessene durchschnittliche Oberflächenrauheit von etwa 6,35 µm (etwa 250 Mikroinch) oder mehr und einem Durchschnitt von Oberflächenpeaks/cm von etwa 15,7 (etwa 40 Peaks/Inch) oder mehr, auf Basis einer oberen Profilometerschwellengrenze von 10,16 µm (400 Mikroinch) und einer unteren Profilometerschwellengrenze von 7,62 µm (300 Mikroinch) aufweist;
- eine leitfähige Zwischenschicht, die eine Oxidschicht ist, die durch Oxidation der schmelzgesprühten Ventilmetalloberfläche durch Erhitzen in Luft oder durch anodische Oxidation hergestellt worden ist, oder eine Hydrid- oder Nitridschicht ist, die hergestellt worden ist, indem die schmelzgesprühte Ventilmetalloberfläche einer hydrierenden oder nitridierenden Behandlung unterzogen worden ist, oder eine schützende und leitfähige Subschicht ist, die auf die schmelzgesprühte Ventilmetalloberfläche aufgebracht worden ist, und
- eine elektrochemisch aktive Oberflächenbeschichtung umfaßt.

26. Gegenstand nach Anspruch 25, bei dem das Substrat ein Ventilmetall wie ein oder mehrere eines Metalls, einer Legierung, einer intermetallischen Mischung, einer Keramik oder eines Cermets umfaßt.

27. Gegenstand nach Anspruch 25 oder 26, bei dem das schmelzgesprühte Metall der Oberfläche ausgewählt ist aus den Metallen, Legierungen und intermetallischen Mischungen von Titan, Tantal, Niob, Aluminium, Zirkonium, Mangan und Nickel.

28. Gegenstand nach Anspruch 27, bei dem die Metalloberfläche eine mittels Profilometer gemessene durchschnittliche Rauheit von etwa 7,62 µm (etwa 300 Mikroinch) oder mehr ohne niedrige Stellen von weniger als etwa 5,33 µm (etwa 210 Mikroinch) aufweist.

29. Gegenstand nach einem der Ansprüche 25 bis 28, bei dem die Oberfläche einen mittels Profilometer gemessenen Durchschnitt an Oberflächenpeaks/cm von mindestens etwa 23,6 (etwa 60 Peaks/Inch), auf Basis einer oberen Schwellengrenze von 10,16 µm (400 Mikroinch) und einer unteren Schwellengrenze von 7,62 µm (300 Mikroinch) aufweist.

30. Gegenstand nach einem der Ansprüche 25 bis 29, bei dem die Oberfläche einen mittels Profilometer gemessenen durchschnittlichen Abstand zwischen dem Maximumpeak und dem Maximumtal von mindestens etwa 25,4 µm (etwa 1000 Mikroinch) aufweist.

31. Gegenstand nach Anspruch 30, bei dem die Oberfläche einen mittels Profilometer gemessenen durchschnittlichen Abstand zwischen dem Maximumpeak und dem Maximumtal von etwa 38,1 µm (etwa 1500 Mikroinch) bis etwa 88,9 µm (etwa 3500 Mikroinch) aufweist.

32. Gegenstand nach einem der Ansprüche 25 bis 31, bei dem die Oberfläche eine mittels Profilometer gemessene durchschnittliche Peakhöhe von etwa 25,4 µm (1000 Mikroinch) oder mehr aufweist.

33. Gegenstand nach Anspruch 32, bei dem die Oberfläche eine mittels Profilometer gemessene durchschnittliche Peakhöhe von etwa 38,1 µm (etwa 1500 Mikroinch) bis etwa 88,9 µm (etwa 3500 Mikroinch) aufweist.

34. Gegenstand nach einem der Ansprüche 25 bis 33, bei dem die Zwischenschicht eine Oxidschicht ist, die in der schmelzgesprühten Oberfläche durch Erhitzen in Luft oder durch anodische Oxidation hergestellt worden ist.

35. Gegenstand nach einem der Ansprüche 25 bis 33, bei dem die Zwischenschicht eine aufgebrachte Subschicht ausgewählt aus elektroplattiertem Platin, elektroabgelagertem Kobaltoxid oder Bleioxid oder einer auf Zinnoxid basierenden Schicht ist.

36. Gegenstand nach einem der Ansprüche 25 bis 35, der eine Elektrode für elektrochemische Verfahren, insbesondere eine sauerstoffentwickelnde Anode ist.

37. Gegenstand nach Anspruch 36, der eine Anode in einer anodisierenden, elektroplattierenden oder elektrolytisch gewinnenden Zelle ist.

38. Gegenstand nach Anspruch 36, der eine Anode zum Elektrogalvanisieren, Elektroverzinnen, zur Natriumsulfatelektrolyse oder Kupferfolienplattierung ist.

39. Zelle für die Elektrolyse einer gelösten Spezies, die in einem Bad dieser Zelle enthalten ist, welche eingetaucht in dieses Bad eine Anode aufweist, die ein beschichteter metallischer Gegenstand gemäß einem der Ansprüche 25 bis 38 ist.

## Revendications

1. Une méthode pour produire un article métallique comprenant un substrat ayant une surface contenant un métal adapté pour une adhésion améliorée d'un revêtement par giclage en fusion de particules d'un métal d'arrêt ayant une taille dans l'intervalle de 20 à 100 micromètres pour produire une surface ayant une rugosité de surface moyenne mesurée au profilomètre d'environ 6,35 micromètres (environ 250 micropouces), ou plus, et environ 15,7 pics moyens en surface par cm (environ 40 pics par pouce), sur la base d'un seuil limite supérieur au profilomètre de 10,16 micromètres (400 micropouces) et d'un seuil limite inférieur au profilomètre de 7,62 micromètres (300 micropouces).

2. La méthode de la revendication 1, dans laquelle le substrat comprend un métal d'arrêt en tant qu'un ou plusieurs d'un métal, alliage, mélange intermétallique, céramique ou cermet.

3. La méthode de la revendication 1 ou 2, dans laquelle le métal giclé en fusion de ladite surface est sélectionné parmi les métaux, alliages, et mélanges intermétalliques de titane, tantale, niobium, aluminium, zirconium, manganèse et nickel.

4. La méthode de la revendication 3, dans laquelle ladite surface en métal a une rugosité de surface moyenne mesurée au profilomètre d'environ 7,62 micromètres (environ 300 micropouces), ou plus, sans points inférieurs à d'environ 5,33 micromètres (environ 210 micropouces).

5. La méthode de n'importe quelle revendication précédente, dans laquelle ladite surface a au-moins environ 23,6 pics moyens en surface par cm (environ 60 pics par pouce), sur la base d'un seuil limite supérieur au profilomètre de 10,16 micromètres (400 micropouces) et d'un seuil limite inférieur au profilomètre de 7,62 micromètres (300 micropouces).

6. La méthode de n'importe quelle revendication précédente, dans laquelle ladite surface a une distance moyenne mesurée au profilomètre entre le pic maximal et la vallée maximale d'au-moins environ 25,4 micromètres (environ 1000 micropouces).

7. La méthode de la revendication 6, dans laquelle ladite surface a une distance moyenne mesurée au profilomètre entre le pic maximal et la vallée maximale d'environ 38,1 micromètres (environ 1500 micropouces) à environ 88,9 micromètres (environ 3500 micropouces).

8. La méthode de n'importe quelle revendication précédente, dans laquelle la surface a une hauteur de pics moyenne mesurée au profilomètre d'environ 25,4 micromètres (environ 1000 micropouces) ou plus.

9. La méthode de la revendication 8, dans laquelle la surface a une hauteur de pics moyenne mesurée au profilomètre d'environ 38,1 micromètres (environ 1500 micropouces) à environ 88, 9 micromètres (environ 3500 micropouces).

10. La méthode de n'importe quelle revendication précédente, dans laquelle la surface est revêtue.

11. La méthode de la revendication 10, dans laquelle ladite surface est revêtue d'un revêtement de surface électrochimiquement actif contenant un métal du groupe du platine, ou un oxyde de métal ou leurs mélanges, en particulier un cristal mixte d'au-moins un oxyde de métal d'arrêt et d'au-moins un oxyde de métal du groupe du platine.

12. La méthode de la revendication 11, dans laquelle ledit revêtement de surface électrochimiquement actif contient au-moins un oxyde sélectionné parmi les oxydes de métal du groupe du platine, la magnétite, la ferrite, et la spinelle d'oxyde de cobalt, le dioxyde de manganèse, le dioxyde de plomb, l'oxyde d'étain, un substituant du platinate, le nickel-oxyde de nickel et le nickel plus les oxydes de lanthanides.

13. La méthode de la revendication 11 ou 12, dans laquelle avant l'application du revêtement de surface électrochimiquement actif une couche d'oxyde d'hydrure ou de nitrure est produite sur la surface giclée par fusion.

14. La méthode de la revendication 11 ou 12, dans laquelle avant l'application du revêtement de surface électrochimiquement actif une sous-couche intermédiaire protectrice et conductrice comme le platine électroplaqué, l'oxyde de cobalt ou l'oxyde de plomb électrodéposé, ou une couche à base d'oxyde d'étain est appliquée sur la surface giclée au plasma.

15. La méthode de n'importe quelle revendication précédente, pour produire une électrode pour des procédés électrochimiques, en particulier une anode dégageant de l'oxygène.

16. La méthode de la revendication 15, pour produire une anode dans une cellule d'anodisation, d'électroplaquage ou d'électrorécupération.

17. La méthode de la revendication 15, pour produire une anode dans l'électrogalvanisation, l'électroétamage, l'électrolyse du sulfate de sodium ou le plaquage de feuille de cuivre.

18. La méthode de préparation d'une surface de métal planaire pour un revêtement à l'adhésion améliorée, laquelle surface a été entaillée, et montre ainsi une perte de planarité, laquelle méthode comprend:
a) le giclage en fusion des entailles de ladite surface avec un métal d'arrêt, de préférence par giclage de plasma, pour établir la planarité de la surface en métal, et ensuite
b) le giclage en fusion de la surface à revêtir, y compris les entailles giclées en fusion, de préférence avec le même métal d'arrêt qu'avant et de préférence par giclage de plasma, avec des particules ayant une taille dans l'intervalle de 20 à 100 micromètres pour donner une rugosité de surface améliorant l'adhésion du revêtement, comme défini dans la revendication 1.

19. La méthode de la revendication 18, dans laquelle lesdites entailles sont premièrement partiellement remplies avec un matériau de soudure et ensuite giclées en fusion avec le métal d'arrêt.

20. La méthode de la revendication 18 ou 19, dans laquelle lesdites entailles sont d'abord fraisées pour donner des entailles fraisées pour le métal appliqué par giclage en fusion.

21. La méthode de préparation d'une surface d'un métal revêtu de forme plane pour un revêtement, laquelle surface a été entaillée à l'usage et montre une perte de planarité, laquelle méthode comprend:
a) soumettre ladite surface de métal revêtue au contact d'un bain fondu contenant un matériau pour enlever ledit revêtement, préférablement en trempant la surface du métal revêtu dans ledit bain fondu;
b) séparer ladite surface de métal dudit bain, en le refroidissant par là même et en enlevant le résidu du bain fondu de là;
c) attaquer intergranulairement la surface à une température élevée et avec un acide fort ou un attaquant caustique;
d) laver ladite surface attaquée en exposant lesdites entailles; et
e) gicler en fusion les entailles de ladite surface avec des particule d'un métal d'arrêt ayant une taille dans l'intervalle de 20 à 100 micromètres, de préférence par giclage de plasma, pour établir la planarité de la surface de métal et donner la rugosité de surface; et
f) par laquelle ladite surface a une planarité de surface plus une rugosité de surface pour une amélioration de l'adhésion du revêtement, comme défini dans la revendication 1, et ladite rugosité de surface est établie à la fois par attaque intergranulaire et giclage de plasma.

22. La méthode de la revendication 21, dans laquelle ladite surface séparée dudit bain fondu pour enlever le revêtement est soumise à une recuite à température élevée pendant une durée suffisante pour donner un réseau intergranulaire d'impuretés au-moins substantiellement continu, comprenant les impuretés à la surface dudit métal.

23. La méthode de la revendication 21 ou 22, dans laquelle lesdites entailles sont d'abord partiellement remplies avec un matériau de soudure et ensuite giclée en fusion avec un métal d'arrêt, de préférence par giclage de plasma.

24. La méthode de la revendication 23, dans laquelle lesdites entailles sont d'abord fraisées pour donner des entailles fraisées pour le métal d'arrêt appliqué par giclage en fusion.

25. Un article métallique revêtu comprenant :
- un substrat ayant une surface contenant un métal adapté pour une adhésion améliorée d'un revêtement par giclage en fusion de particules d'un métal d'arrêt ayant une taille dans l'intervalle de 20 à 100 micromètres pour produire une surface ayant une rugosité de surface moyenne mesurée au profilomètre d'environ 6,35 micromètres (environ 250 micropouces), ou plus, et environ 15,7 pics moyens en surface par cm (environ 40 pics par pouce), sur la base d'un seuil limite supérieur au profilomètre de 10,16 micromètres (400 micropouces) et d'un seuil limite inférieur au profilomètre de 7,62 micromètres (300 micropouces);
- une couche intermédiaire conductrice qui est une couche d'oxyde produite par l'oxydation de la surface de métal d'arrêt giclée en fusion par chauffage dans l'air ou par oxydation anodique ou une couche d'hydrure ou de nitrure produite en soumettant la surface de métal d'arrêt giclée en fusion à un traitement d'hydruration ou de nitruration; ou est une sous-couche protectrice et conductrice appliquée sur la surface de métal d'arrêt giclée en fusion; et
- un revêtement de surface électrochimiquement actif.

26. L'article de la revendication 24, dans lequel le substrat comprend un métal d'arrêt en tant qu'un ou plusieurs d'un métal, alliage, mélange intermétallique, céramique ou cermet.

27. L'article de la revendication 25 ou 26, dans lequel le métal giclé en fusion de ladite surface est sélectionné parmi les métaux, alliages, et mélanges intermétalliques de titane, tantale, niobium, aluminium, zirconium, manganèse et nickel.

28. L'article de la revendication 26, dans lequel ladite surface en métal a une rugosité de surface moyenne mesurée au profilomètre d'environ 7,62 micromètres (environ 300 micropouces), ou plus, sans points inférieurs à moins d'environ 5,33 micromètres (environ 210 micropouces).

29. L'article de n'importe quelle revendication 25 à 28, dans lequel ladite surface a au-moins environ 23,6 pics moyens en surface par cm (environ 60 pics par pouce), sur la base d'un seuil limite supérieur au profilomètre de 10,16 micromètres (400 micropouces) et d'un seuil limite inférieur au profilomètre de 7,62 micromètres (300 micropouces).

30. L'article de n'importe quelle revendication 25 à 29, dans lequel ladite surface a une distance moyenne mesurée au profilomètre entre le pic maximal et la vallée maximale d'au-moins environ 25,4 micromètres (environ 1000 micropouces).

31. L'article de la revendication 30, dans lequel ladite surface a une distance moyenne mesurée au profilomètre entre le pic maximal et la vallée maximale d'environ 38,1 micromètres (environ 1500 micropouces) à environ 88,9 micromètres (environ 3500 micropouces).

32. L'article de n'importe quelle revendication 25 à 31, dans lequel la surface a une hauteur de pics moyenne mesurée au profilomètre d'environ 25,4 micromètres (environ 1000 micropouces) ou plus.

33. L'article de la revendication 32, dans lequel la surface a une hauteur de pics moyenne mesurée au profilomètre d'environ 38,1 micromètres (environ 1500 micropouces) à environ 88,9 micromètres (environ 3500 micropouces).

34. L'article de n'importe quelle revendication 25 à 33, dans lequel la couche intermédiaire est une couche d'oxyde produite dans la surface giclée en fusion par chauffage dans l'air ou par oxydation anodique.

35. L'article de n'importe quelle revendication 25 à 33, dans lequel la couche intermédiaire est une sous-couche appliquée, sélectionnée parmi le platine électroplaqué, l'oxyde de cobalt ou l'oxyde de plomb électrodéposé, ou une couche à base d'oxyde d'étain.

36. L'article de n'importe quelle revendication 25 à 35, qui est une électrode pour des procédés électrochimiques, en particulier une anode dégageant de l'oxygène.

37. L'article de la revendication 36, qui est une anode dans une cellule d'anodisation, d'électroplaquage ou d'électrorécupération.

38. L'article de la revendication 36, qui est une anode dans l'électrogalvanisation, l'électroétamage, l'électrolyse du sulfate de sodium ou le plaquage de feuille de cuivre.

39. Une cellule pour l'électrolyse d'une espèce dissoute contenue dans un bain de ladite cellule et ayant immergée dans ledit bain une anode qui est un article métallique comme revendiqué dans n'importe quelle revendication 25 à 38.
